

Aug. 30, 1927.

L. HONIGMANN ET AL

1,640,502

DISTILLATION AND COOKING OF CARBONACEOUS MATERIALS

Filed Jan. 7, 1927



L. Honigmann and F. Bartling  
inventor

by: Marks & Clark  
Atty's.

Patented Aug. 30, 1927.

1,640,502

# UNITED STATES PATENT OFFICE.

LUDWIG HONIGMANN, OF BICHLERHOF, BAD TOLZ, AND FRIEDRICH BARTLING, OF MUNICH, GERMANY.

## DISTILLATION AND COOKING OF CARBONACEOUS MATERIALS.

Application filed January 7, 1927, Serial No. 159,700, and in Germany November 26, 1925.

In many furnaces and similar devices for the drying and the distilling of fine granular material, this material is spread out in a thin layer on a surface and exposed to the action of heat, the surface bearing the layer of material being usually passed through a heating or re-action chamber if the drying process is to be carried out in a continuous manner. Although it is also known that in the case of certain kinds of material to be dried, the spreading out in a thin and uniform layer is advantageous, in that the heating action and also the withdrawal of the vapours and gases are facilitated, it has hitherto been held that the diminution in the thickness of the layer should not be carried beyond a certain limit, as otherwise the operation ceased to be economical owing to the smallness of the quantity of material treated per unit of time. By "a very thin layer" in this connection would be understood a layer having a thickness of a few centimetres. The factory treatment of material to be dried was regarded as impossible in layers of less than 1.5 cm.

Exhaustive experiments carried out by the inventors have yielded the surprising result that it is possible to work advantageously with layers, the thickness of which is of an order of magnitude altogether different from what has hitherto been regarded as possible. Experiments, particularly with furnaces with a revolving annular horizontal hearth, hereinafter referred to as revolving ring plate furnaces, wherein upon the revolving hearth quite uniform layers are spread of a thickness amounting to not more than a few millimetres, have given altogether astonishing results, in that the output attained with the furnace has amounted to twenty times, and more than twenty times, the output reached with layers of a thickness of a few centimetres. In the case of fine granular material, the spreading of such thin layers presents no difficulty at all. The essential advantage of such thin layers consists in the direct and almost instantaneous action of the heat. The layer can in this manner be successfully passed through a comparatively small furnace chamber at a high speed, thus effecting a complete heat treatment of the material. Thus for example wet peat having a water content of from 50 to 55 per cent, in a single

revolution of a small experimental furnace, was not only thoroughly dried, but also coked and freed from oil. The entire drying and distillation process was completely finished in a single revolution of the furnace, which only occupied 28 seconds and comprised a path of about 4 metres in length.

Accordingly a process according to the invention for the drying or coking of fine granular material by heat treatment in a thin layer is characterized by the fact that the material is spread out into layers the thickness of which amounts to fractions of a centimetre.

In a preferred constructional form of the new process, layers of such thickness are employed in continuous operation in connection with very high speed revolving plate furnaces.

The result is to increase the output of each unit of heating surface per unit of time to a multiple of what it would be under ordinary circumstances. From this there follows the further advantage of being able to employ very small and high speed rotating furnaces, revolving ring plate furnaces for example, whereby for the same output there is a very considerable saving in space, expenditure of time, labour, and heating costs. Below are described the experiments by which the inventors have established the great superiority of their process over the known process.

Upon a heated steel plate of a particular size were spread out in succession accurately weighed quantities of fine granular lignite in layers of different thicknesses, in such a way that the material completely covered the heating surface in an exactly uniform layer. Each layer of material was left on the heating surface until completely dried and then removed. The duration of each drying operation was accurately determined. First of all a weighed quantity was spread out in a layer 15 millimetres in thickness, corresponding to the smallest thickness of layer hitherto regarded as practicable. After the complete drying of this quantity, three times the same quantity by weight of moist coal was divided, firstly into 15 parts, secondly in to 7.5 parts, and finally into 5 parts.

Thereupon, of the quantity divided into 15 parts, the 15 parts were taken in succession one at a time and spread on the plate,

giving on each occasion a layer 1 millimetre in thickness, and each of these 15 layers was dried with similar heating until it was entirely free from water. In the same manner the two remaining quantities were spread out and dried, one in 7.5 layers each 2 millimetres thick and the last in 5 layers each 3 millimetres thick.

The accurately recorded results prove that 10 the same quantity of coal, always spread out with similar heating, first in a layer of 15 millimetres thick, required 15.02 times as long as the same quantity of coal with the same water content when spread out in a 15 layer only 1 millimetre thick, 14.13 times as long as when spread out in a layer 2 millimetres thick, and 8.55 times as long as when spread out in a layer 3 millimetres thick.

Hence for a layer 1 millimetre thick the 20 output was 15.02, 2 millimetres thick the output was 14.13, 3 millimetres thick the output was 8.55 times as great as in the case of a layer 15 millimetres thick.

The present process is however of particular value for the distillation of bituminous substances. It was not obvious that such thin layers, in connection with a revolving ring plate furnace, could have a particularly advantageous action when employed for 30 the distillation. Hitherto the distillation has almost universally been effected in compact masses, and the idea of a very thin spreading of the material to be distilled is particularly fruitful in connection with a device by which 35 this thin layer traverses a path of quite definite length in a quite definite time through a heating chamber, for it is clear that the distillation in such a thin layer completely breaks with the methods hitherto usual, and 40 that in consequence of the great output of the heating surface per unit of time it must always be carried out continuously and with a certain quickness in order to be successful. For this purpose, however, it is just the 45 revolving ring plate furnace that presents the best means. This furnace also renders it possible to effect the spreading out and the discharging of the fine-grained and ultimately pulverulent material in an advantageous 50 manner, whereas the scraping means or the like previously used failed completely. It is clear that the suggestions (1) of employing, for the distillation, in order to produce half-coke and high grade tar oils, a revolving ring plate furnace, upon the movable heat exchanging surfaces of which (2) the 55 material is spread out in an extremely thin layer, presents technology with altogether new methods of low temperature coking.

60 In the distillation of bituminous substances it is of tremendous importance that the entire material to be distilled should be worked through quite uniformly, that is to say, that the material during the distillation process, should be exposed to the same

temperature in all its parts. The inventors have ascertained that this uniform treatment is only possible in its entirety when layers of material are employed which are very thin, that is to say, less than 1 centimetre in thickness, as only then can it be guaranteed that the heating action is the same upon all parts of the material. With thicker layers the bottom layer of material undergoing distillation covering the heating surface of the furnace is unavoidably more strongly heated than the layer lying above it. Furthermore, the employment of such thin layers has also the further immense advantage that the escape of the gases from the material undergoing distillation can take place immediately upon the attainment of the corresponding degree of heat without any hindrance. By this means the distillation process is very considerably shortened, that is to say, 85 each square metre of heating surface will attain a very considerably greater output per unit of time.

This uniform treatment of the material undergoing distillation, is of such great importance on account of the fact that only the uniformity of the temperature action upon all parts of the material makes it possible for the whole of the final product obtained, that is to say, the whole of the coke or half-coke accruing, to be of the same quality in all its parts, that is to say, for all its parts to contain the same proportion of gas.

According to the treatment of these parts, besides the uniformity of the final product, that is, of the half-coke, the further result is obtained that the oils obtained by the distillation process from all parts of the material undergoing distillation are of the same quality throughout, never varying during 105 the process.

It is also quite obvious that the known process, according to which the oil-carrying vapours that become free in the various stages of the distilling process are separately collected and separately worked up according to their percentage of valuable substances, undergoes considerable improvement by the method of treatment according to the present invention. As is known, in a revolving ring plate furnace or any similar furnace arrangement the furnace space above the travelling plate may be divided into zones in which the various grades of distillation gases are separately collected. Now when working with the relatively thick layers that have hitherto been usual in distillation, a clean separation of these various grades of distillation gases obviously becomes less possible, the thicker the layer is, 125 for, as stated, the thickness of the layer prevents a simultaneous and completely uniform treatment of the material. The portions of the material adjacent to the heat exchanging surface are treated more quick- 130

ly. Thus the gases of similar composition rise from the various superposed layers of material at different times, distillation gases of different qualities mixing with one another, and the separate collection is for the most part prevented or at least impaired.

The employment of a minimum thickness of layer, in connection with a revolving ring plate furnace, renders possible quite generally a remarkably advantageous adjustability of the distilling and coking process. The products to be obtained may be determined in advance as regards their kind and quality, as soon as the two determining factors here are regulated, namely, (1) the desired maximum temperature at which distillation takes place, and (2) the duration of the action of this maximum temperature upon the material undergoing distillation.

20 By the spreading of a more or less thin layer, by regulating the speed of the working plate of the revolving furnace, and also by regulating the heating of this rotating working plate, the possibility is provided in practice of determining at will the quality of the half-coke accruing, and also the quality of the oils accruing.

In the accompanying drawings one constructional example is illustrated of a furnace in which the new process can be carried out. In these drawings—

Fig. 1 shows in sectional elevation through the centre such a furnace with an annular revolving hearth,

Fig. 2 shows on a larger scale part of the working plate of the hearth with the layer resting thereon.

In the constructional example illustrated, *a* is an annular furnace crown, the furnace chamber of which is open at the bottom and is closed by the annular hearth *b*.

In the constructional example shown, there are arranged in the crown of the furnace annular heating flues *c*, which serve to heat the hearth plate from below. Further heating flues *d* may also be employed for heating the hearth plate from above.

The revolving hearth consists of two superposed hearth plates *e* and *f* rigidly connected with one another. The lower plate *e* serves to close the furnace from the exterior and the upper plate *f* is the actual working hearth and serves for the reception of the material undergoing treatment. The interval of space between the plates *e* and *f* is made so great that radiant heating from below by the lateral heating flues *c* is rendered possible. The two hearth plates *e* and *f* rigidly connected with one another rest by means of a carrying ring *g* upon a carriage *h*, which runs upon a railway *i*. The carriage *h* carries a ring of teeth *k*, which can be rotated by means of any convenient driving device *l*. For the spreading

there serves a spreading device *m*. The latter comprises a spreading box *n*, which is open at the bottom and to which the material to be treated is supplied through a pipe *o*. Preferably the filling box *n* slides with its lateral edges upon lateral ribs *f'* on the hearth plate *f*. A knife-like ledge *p* is adjustably secured to the filling box *n* in such a way as to extend downwards almost to the sole of the hearth. The ledge is so adjusted that between its lower edge and the sole of the hearth there remains a gap of a few millimetres. By this means the thickness of the layer spread is determined. The gases and vapours rising from the material may be drawn off from the furnace through suction tubes *q*. When it is a question of the distillation of bituminous substances, a plurality of suction tubes *q* may be arranged at such positions that the various fractions of the oils obtained are collected separately. The heating flues *c* and *d* may be heated by any convenient heating gases.

When using the furnace for the production of a half-coke for example from peat, lignite, or any other bituminous substance, the fine-grained pulverulent or similar material is shot in through the tube *o* and falls out of the filling box *n* on to the hearth *f*. The hearth *f*, moving forward underneath the filling box *n*, takes with it a layer of material a few millimetres thick, the excess being scraped off by the ledge *p*. During its passage through the furnace the material is distilled, the heating action being effected with extreme quickness in consequence of the exceptional thinness of the layer. Before the material travelling through the furnace chamber returns to the spreading point the coking is finished to the desired extent. The material may therefore be discharged by any suitable means shortly before it reaches the filling point *m* again.

What we claim is:—

1. In the process of distilling and coking solid carbonaceous material on annular revolving hearths, the steps which comprise maintaining a layer of such material on the hearth in a thickness less than one centimeter and subjecting the material to a coking heat until coked.

2. In the process of distilling and coking solid carbonaceous material on annular revolving hearths, the steps which comprise maintaining a layer of such material on the hearth in a thickness less than one centimeter and subjecting the material to a coking heat until coked, said heat being sufficient to complete the coking in one revolution of the hearth.

3. In the process of distilling and coking solid carbonaceous material on annular revolving hearths, the steps which comprise maintaining a layer of such material on the hearth in a thickness of about one to three

millimeters and subjecting the material to a coking heat until coked.

4. In the process of distilling and coking solid carbonaceous material on annular revolving hearths, the steps which comprise maintaining a layer of such material on the hearth in a thickness of about one to three millimeters and subjecting the material to

a coking heat until coked, said heat being sufficient to complete the coking in one <sup>10</sup> revolution of the hearth.

In testimony whereof we have signed our names to this specification.

LUDWIG HONIGMANN.  
FRIEDRICH BARTLING.